

## UNITED STATES PATENT OFFICE

2,413,365

CLEANING COMPOSITION FOR ALUMINUM  
AND ALUMINUM ALLOYSLowell R. McCoy, Detroit, Mich., assignor to  
Wyandotte Chemicals Corporation, Wyandotte,  
Mich., a corporation of MichiganNo Drawing. Application April 13, 1944,  
Serial No. 530,939

8 Claims. (Cl. 252—142)

1

It is an object of this invention to prepare a cleaning composition in dry or substantially dry form, which when placed in solution will afford an excellent cleaner for aluminum and its alloys, preparatory to spot welding. While the composition inherently has some cleaning ability for various metals, its primary utility is for the purpose specified.

It is also an object to prepare a cleaning bath and to employ a method wherein this composition is employed.

It is necessary to remove the oxide films formed during natural oxidation and heat treatment of aluminum and its alloys, which films are non-uniform and of high resistance in relation to that of the metal. It is now quite generally agreed that in spot welding of aluminum alloys for aircraft structures the surface film plays an extremely important part in determining weld quality. One authority has stated, "it appears that at least 75 per cent of the troubles experienced with surface spitting, weld spitting, irregularity in weld shape and the extent of electrode pickup can be attributed to improper surface preparation." Various methods both chemical and mechanical have been employed for removing oxide films from aluminum surfaces preparatory to spot welding. Each, however, leaves much to be desired.

Most of the oxide-removing solutions in use today fall into three categories: (1) hot or cold dilute acids (2) cold concentrated acids and (3) alkaline compositions. Hydrofluoric acid which is an example of (1) requires time control within a few seconds. Otherwise formation of film due to chemical reaction will result upon overtreatment, which film is injurious to good welding. Acids like phosphoric take too long a time unless traces of fluorides are present. The concentration of the latter is, however, almost impossible to control by any simple method. The alkaline type is not satisfactory except as degreasers because the strong alkalies attack aluminum and give highly erratic results.

Hydrofluosilicic acid, i. e.  $H_2SiF_6$ , which can be purchased commercially at a low cost in concentrations of 27-30% has been employed at about 3 and 4% by volume concentrations in baths, preferably in about 3%. The pH value based thereon is kept between 0.95 and 0.90 during the entire treating time of 6 to 10 minutes at room temperature. This method using this acid has several advantages as is readily apparent from the above statements. Also there is less danger of overtreatment as is the case with most acids. However, there are disadvantages with all liquid acids such as the difficulty of handling, weight of inert solvent therein, cost of containers and chances of breaking them.

A mixture of ammonium silico fluoride and

2

sodium acid sulfate, i. e. niter cake, when placed in an aqueous solution, I have found, liberates free fluosilicic acid. But this solution possesses the disadvantage that sodium silico fluoride is precipitated in dilute solution, such as a 3% solution of said components in stoichiometric proportions. By the addition of ammonium sulfate, I have determined that all but a negligible part of this precipitation is prevented. The addition of a wetting agent such as an alkyl-aryl sodium sulfonate in small amounts promotes both rapidity and effectiveness of the action of the cleaner. Where a wetting agent is not employed, the resistance of the treated surface is higher and more difficult of duplication than in the case where it is present under the same condition.

Various wetting agents may be employed such as the alkali metal or basic nitrogen salts of sulfonated oils, sulfonated primary and secondary alcohols, sulfated amides, sulfated esters of mono-acid dibasic acids and higher alkyl-aryl sulfonates. The last type does not hydrolyze easily and is, therefore, stable in acid solutions.

My preferred composition is a mixture of 18.5% (all percentages hereinafter given being by weight unless otherwise specified) ammonium silicofluoride, 25% niter cake, 52.5-54.5% ammonium sulfate and 2-4% of a higher alkyl-aryl sodium sulfonate, such as a kerosene-benzene sodium sulfonate. Niter cake is a crude sodium sulfate containing some bisulfate and very small amounts of other substances. But pure sodium acid sulfate will serve the purpose. In this mixture the first two recited components are in approximately stoichiometric proportions. That is to say, the ammonium silicofluoride and sodium sulfate are present in such proportions, based on their respective molecular weights, as to react according to the following chemical equation, producing fluosilicic acid:



A suitable concentration is 8 ounces of the composition to a gallon of water. The following table sets out times of treatment in the bath of said solution at various temperatures.

Table

| 50            | Thickness<br>in inches of<br>"Alclad<br>24 S-T" <sup>1</sup> | Time of treatment in<br>minutes. | Temperature of bath |           |           |           |
|---------------|--------------------------------------------------------------|----------------------------------|---------------------|-----------|-----------|-----------|
|               |                                                              |                                  | 60°<br>F.           | 70°<br>F. | 80°<br>F. | 90°<br>F. |
| 0.020.....    |                                                              | 8                                | 6                   | 5         | 4         |           |
| 55 0.051..... | do.....                                                      | 10                               | 8                   | 6         | 5         |           |

<sup>1</sup> "Alclad 24 S-T" is an alloy consisting of a base of aluminum alloy having good physical properties protected from corrosion by a layer of very pure aluminum on both surfaces of the sheet, the cladding constituting 5-10% of the thickness of the sheet. The composition of the base metal is 93.7% Al, 4.2% Cu, 0.6% Mn and 1.5% Mg.

Such treating times remain as indicated until the concentration (determined by the titration using N/1 NaOH and methyl orange as indicator) falls to 1.5 gm/100 cc.

The advantage of using this aforesaid ratio of constituents in the dry mixture is that the same proportions can be added for repleting. The concentration of the solution can be varied widely without much change of time treatment.

The concentration of the treating bath can vary from substantially 1.5% up to 10% depending somewhat on the temperature; but for high temperatures the upper limit should not exceed 8%.

There are various methods in which this mixture can be employed in solution. By one mode aluminum objects are immersed in a solution at room temperature containing approximately 6% by weight of the mixture for varying lengths of time depending upon the thickness of the metal as shown in the table. The reason for the effect of thickness of the metal upon the time required for treatment may be the presence of the thicker coating of oxide upon the thicker gages, due to longer time required for heat treatment. Or it may be due to the greater amount of copper in the cladding of the thinner metal due to the shorter distance through which it must diffuse from the base metal to the surface of the cladding. Traces of copper accelerate the action of the acid upon the aluminum. It may be both factors are responsible. Immediately following this treatment the objects are thoroughly rinsed and dried.

In laboratory tests, the aluminum so treated has been found to be suitable for spot welding after as much as a week has elapsed since said treatment. A longer period results in a change of the surface believed to be the result of oxidation. In factory practice, however, where chances of the object being contaminated through handling, etc., are much greater, a twenty-four hour limit between treatment and spot welding is to be preferred.

The above description and examples are illustrative only. Any modification of or variation therefrom which conforms to the spirit of the invention is intended to be included within the scope of the claims.

I claim:

1. A metal cleaning composition, particularly adaptable for removing oxide films from aluminum and its alloys, comprising ammonium silicofluoride and sodium acid sulfate both present in substantially stoichiometric proportions for re-

55

action with each other, and ammonium sulfate present in sufficient amount to inhibit the formation of a precipitate in water solutions of said composition.

5 2. A metal cleaning composition, particularly adaptable for removing oxide films from aluminum and its alloys, comprising by weight 18% ammonium silicofluoride, 52.5-54.5% ammonium sulfate, 25% sodium acid sulfate and the balance a sulfonated organic compound wetting agent.

3. In the process of removing oxide films from aluminum and its alloys, the step of applying to the surface thereof an aqueous solution comprising ammonium silicofluoride and sodium acid sulfate both present in stoichiometric proportions for reaction with each other, water, and ammonium sulfate present in sufficient amount to inhibit the formation of a precipitate in said solution.

15 10 4. In the process of removing oxide films from aluminum and its alloys the step of applying to the surface thereof an aqueous solution comprising water and a mixture of, by weight 18% ammonium silicofluoride, 25% sodium acid sulfate, and 52.5-54.5% ammonium sulfate.

15 15 5. In the process of removing oxide films from aluminum and its alloys, the step of applying to the surface thereof an aqueous solution comprising water and a mixture of, by weight 18% ammonium silicofluoride, 25% sodium acid sulfate, 52.5-54.5% ammonium sulfate, and the balance a sulfonated organic compound wetting agent.

20 20 6. A metal cleaning solution comprising water and a cleaning composition forming 1-10% by weight thereof and comprising ammonium silicofluoride and sodium acid sulfate both present in substantially stoichiometric proportions for reaction with each other, and ammonium sulfate present in an amount sufficient to inhibit the formation of a precipitate in said solution.

25 25 7. A metal cleaning solution comprising by weight a 1-10% aqueous solution of 18% ammonium silicofluoride, 25% sodium acid sulfate, 52.5-54.5% ammonium sulfate, and the balance a sulfonated organic compound wetting agent.

30 30 8. The process of cleaning aluminum and aluminum alloys which comprises treating the surface thereof with a 1-10% by weight aqueous solution of a mixture of 18% ammonium silicofluoride, 25% sodium acid sulfate and 52.5-54.5% ammonium sulfate, at a temperature of 60-90° F. and for a period of 4 to 10 minutes.

LOWELL R. McCOY.